



for example made of polyester fibres/cotton, polyester fibres/spun rayon, polyacrylonitrile fibres/spun rayon, polyester fibres/linen, polyester fibres/wool or polyamide fibres/cotton etc.

The preparation of the compounds of the Formula I by reacting bis-organic tin oxides of the Formula II, for example bis-tributyl tin oxide, with carboxylic acids of the Formula III, for example  $\beta$ -tetrafluoro-cyclobutyl acrylic acid or methyl-tetrafluoro-cyclobutyl acrylic acid may be carried out according to known processes in a suitable organic solvent such as benzene, toluene and xylene. The reaction proceeds at elevated temperature, expediently at the boiling temperature of the solvent under reflux, whereby according to the reaction desired, about 2 mols of the carboxylic acid of the Formula III per mol of the bis-organic tin oxide of the Formula II are used. The water formed during condensation was eliminated together with the solvent by azeotropic distillation. The substance left after distilling off the solvent may be used, if desired, directly, without any further purification, for the antimicrobially finishing according to the invention.

The tin-organic compounds of the Formula I are soluble in many organic solvents. Particularly suitable solvents with regard to the textile application of these compounds are lower aliphatic alcohols, especially those having 1 to 4 carbon atoms. The tin-organic compounds according to the invention are also soluble in an aqueous, alkaline medium, for example in aqueous solutions of alkali hydroxides, alkali carbonates or -bicarbonates. When being applied onto textiles, they may therefore be applied from organic solvents, from mixtures of solvent and water and at pH-values above 7 from aqueous solutions or emulsions, for example those consisting of chloro- or fluorohydrocarbons with water or alcohol. For the antimicrobial finishing of textiles there are generally used solutions which show a content of about 10 to 100 g., preferably 15 to 40 g., of the tin-organic compounds of the Formula I per liter of bath. This concentration of the finishing baths mostly insures an effective amount of deposit depending on the squeezing out effect. The minimum of the effective amount required is about 0.3%, calculated on the goods weight. There is no upper limit for the amounts of tin-organic compounds to be applied. However, an amount to be applied exceeding about 5% cannot be considered practical for economical reasons.

For the antimicrobial finish of textiles, the tin-organic compounds of the Formula I may be used as such and together with other finishing and binding agents. It is also possible to apply the tin-organic compounds together with optical brighteners or antistatically effective agents. For finishing textiles which consist of cellulose fibres or contain cellulose fibres, the tin-organic compounds are expediently applied onto the textile material with crease-resistant finishing agents. In this process—especially in the case of cross-linking under dry conditions—good boil-proof fungistatic effects can be achieved. The tin-organic compounds may also be used in the known cross-linking processes of textiles in the presence of more or less amounts of water. Particularly advantageous is the use of tin-organic compounds together with finishing agents which are cross-linking in an alkaline medium. The tin-organic compounds may also be used in the dyeing of textiles and may be added for example to the dyestuff bath or printing paste. By this way, antimicrobial effects are simultaneously obtained with the dyeing or printing. A special advantage is the application of the tin-organic compounds together with dyestuffs which can be fixed in an alkaline medium. It is furthermore possible to apply the tin-organic compounds onto the textile material together with hydrophobing, oleophobing and flame-proof finishing agents.

The tin-organic compounds of the Formula I may be applied onto the good to be finished in any manner desired, for example by padding, slop padding, spraying,

doctoring or according to the exhaustion process. The textiles treated with the solutions or dispersions of the tin-organic compounds are dried at room temperature or elevated temperature and expediently heated for about 1 second to 5 minutes up to high temperatures. The choice of the temperature depends on the heating time and on the textile material. There are generally used temperatures in the range of about 110 to 220° C. It has turned out advantageous to subject the textiles treated with the tin-organic compounds of the Formula I and dried, with solutions of diluted alkalis or to apply the compounds of the Formula I to textiles pretreated with alkalis and alkaline reaction.

It is also possible to incorporate the tin-organic compounds according to the invention into pastes, pigment mixtures and the like for coating purposes. The use of the tin-organic compounds together with plastic dispersions, such as polyacrylate, polyurethane, butadiene-co-polymer, polyvinylacetate dispersions or natural latex, is particularly important, if floor covering, for example carpets, needle felts, mats or fleeces shall be finished fungistically and bacteriostatically.

In the following examples parts and percentages are by weight unless stated otherwise.

The antimicrobial efficiency of the textile finishes in the following examples was tested according to the method described in the periodical "Textilveredlung" 5 (1970), pp. 12 to 14. For this purpose, Petri dishes of plastics were fed each with 20 ml. of malt extract-dextrose-agar and the germs were applied onto the solidified surface as inoculating layer. The ends of the layers were covered with a test cloth (2 x 2 cm.) of the finished good. After an incubation time of 8 days at 28° C., the growth of the germs on the textile material and in its surroundings (incubation zone) was estimated as follows:

| Findings                                                                                                                             | Mark |
|--------------------------------------------------------------------------------------------------------------------------------------|------|
| The agar layer over the fabric sample shows the same growth intensity of the test germ as the surroundings.....                      | 1    |
| On the agar layer over the sample only some colonies are growing; inhibition of growth in contradistinction to the surroundings..... | 2    |
| 45 The agar layer over the fabric sample does not show any colonies of microorganisms.....                                           | 3    |
| 40 No growth on the agar layer above the sample; an inhibition zone not larger than 2 mm. is clearly visible around the sample.....  | 4    |
| 40 Around the fabric sample there is an inhibition zone of more than 2 mm.....                                                       | 5    |

50

### EXAMPLE 1

Fabric samples made of polyamide fibres were impregnated in each case with the following solutions:

Solution A:

1.5 parts of tributyl-tin- $\beta$ -tetrafluorocyclobutyl acrylate,  
24.5 parts of water,  
74.0 parts of isopropanol.

Solutions B:

1.5 parts of tributyl-tin- $\beta$ -(methyl)-tetrafluorocyclobutyl acrylate,  
24.5 parts of water,  
74.0 parts of isopropanol.

Solution C:

1.5 parts of triphenyl tin- $\beta$ -(methyl)-tetrafluorocyclobutyl acrylate,  
24.5 parts of water,  
74.0 parts of isopropanol.

Solution D (comparison):

1.5 parts of tributyl tin oxide,  
24.5 parts of water,  
74.0 parts of isopropanol.

The squeezing off effect was 50% by weight.

After pad-dyeing the fabric was dried and fixed by heating for one minute to 180° C. The textiles finished with the solutions A to C have an excellent fungistatic and a bacteriostatic effect.

The results obtained from the tests with regard to growth inhibition against the dermatomyces *Trichophyton mentagrophytes* 109 and the soil fungus *Aspergillus niger* 533 after three washing processes with a household washing machine were compiled in Table I.

TABLE I

| Solution | Growth inhibition (mark)  |                          |
|----------|---------------------------|--------------------------|
|          | <i>Trichophyton ment.</i> | <i>Aspergillus niger</i> |
| A-----   | 3                         | 3                        |
| B-----   | 5                         | 3                        |
| C-----   | 5                         | 4                        |
| D-----   | 1                         | 1                        |

## EXAMPLE 2

The samples of a polyacrylonitrile fabric were treated in each case with the following solutions:

Solution A:

Tributyl-tin- $\beta$ -(methyl)-tetrafluoro-cyclobutyl acrylate in isopropanol/water (3:1 parts by volume).

Solution B:

Triphenyl tin- $\beta$ -(methyl)-tetrafluoro-cyclobutyl acrylate in isopropanol/water (3:1 parts by volume) and

Solution C (comparison):

Tributyl tin oxide in isopropanol/water (3:1 parts by volume).

The squeezing off effect was 50% by weight.

The fabric samples were dried at 100° C. and fixed for one minute at 150° C. The finishes prepared with the solutions A and B have excellent fungistatic effects against dermatomycetes and soil fungi and yeast.

The following Table 2 resumes the antimicrobial effects after three washing processes in a washing machine:

TABLE 2

| Solution | Growth inhibition (mark)  |                              |                             |                              |
|----------|---------------------------|------------------------------|-----------------------------|------------------------------|
|          | <i>Trichophyton ment.</i> | <i>Candida albicans</i> St 1 | <i>Candida albicans</i> 604 | <i>Aspergillus niger</i> 533 |
| A-----   | 3                         | 3                            | 3                           | 3                            |
| B-----   | 3                         | 3                            | 3                           | 3                            |
| C-----   | 1                         | 1                            | 1                           | 1                            |

## EXAMPLE 3

The samples of a cotton poplin were impregnated with solutions of the following composition indicated:

Solution A:

150 g./l. of dimethylol-dihydroxy-ethylene-urea (50%),  
15 g./l. of Mg-chloride,  
15 g./l. of tributyl tin- $\beta$ -tetrafluoro-cyclobutyl acrylate.

Solution B:

150 g./l. of dimethylol dihydroxy-ethylene-urea (50%),  
15 g./l. of Mg-chloride,  
15 g./l. of tributyl tin-(methyl)-tetrafluoro-cyclobutyl acrylate.

Solution C:

150 g./l. of dimethylol-dihydroxy-ethylene urea (50%),

15 g./l. of Mg-chloride,  
15 g./l. of triphenyl tin- $\beta$ -(methyl)-tetrafluoro-cyclobutyl acrylate.

Solution D (comparison):

150 g./l. of dimethylol-dihydroxy-ethylene urea (50%),  
15 g./l. of Mg-chloride,  
15 g./l. of tributyl tin oxide.

10 The squeezing off effect was 50% by weight.

After pad-dyeing the fabric was dried and fixed by heating for one minute to 180° C. The textiles finished with the solutions A to C have an excellent fungistatic and a bacteriostatic effect.

15 As solvent there is used a mixture of 3 parts by volume of isopropanol and 1 part by volume of water.

After pad-dyeing the samples were dried at 100° C. on a stretching frame and then condensed for 5 minutes at 150° C. The samples of the finished fabrics show a marked fungistatic effect against dermatomycetes, soil fungi and blastomycetes and a bacteriostatic effect against *Staphylococcus aureus*.

After two processes in a washing machine, a clear inhibition of growth of *Trichophyton mentagrophytes* (dermatomycetes) and *Aspergillus niger* (soil fungus) could be demonstrated in the case of the samples A to C. On the sample D, however, no efficiency of the finish was observed. Whereas the tin-organic compounds in the solutions A to C have practically no influence on the dry creasing angles of the fabrics, the tributyl tin oxide of the sample D causes a considerable diminution of the dry crease angle.

## EXAMPLE 4

35 Samples of a cotton fabric were impregnated in each case with a bath consisting of

Solution A:

10 g./l. of tributyl tin- $\beta$ -tetrafluoro-cyclobutyl acrylate and,

Solution B:

10 g./l. of tributyl tin- $\beta$ -tetrafluoro-cyclobutyl acrylate.

45 squeezed off until reaching a weight increase of 70% and dried at 100° C. Isopropanol/water (3:1 parts by volume) is used as solvent. The dried fabric samples were then treated with 5 g./l. of sodium hydroxide solution (32%), rolled together and packed in a foil. After storing for 18 hours in this state, the samples were rinsed, neutralized and dried.

50 The fabrics have an excellent fungistatic effect against dermatomycetes, yeasts and soil fungi and a bacteriostatic effect. It must be mentioned that these samples show after two processes in washing machines a strong inhibition of the growth of the fungi on the fabric sample and at the periphery of the sample in the case of *Trichophyton mentagrophytes*, *Candida albicans* and *Aspergillus niger*, furthermore in the case of *Staphylococcus aureus*.

## EXAMPLE 5

60 A polyester fibre fleece was impregnated on the padding machine with a bath which contained

65 25 parts of a 42% aqueous dispersion of a copolymer consisting of 52% of butyl acrylate, 25% of acrylonitrile, 21% of styrene and 2% of acrylamide,

2 parts of tributyl tin- $\beta$ -(methyl)-tetrafluorocyclobutyl acrylate and

70 33 parts of isopropanol.

After squeezing off to reach a weight increase of 50%, the whole was dried and condensed for 7 minutes at 130° C. The reinforced fleece showed in the test a fungistatic and bacteriostatic effect against *Trichophyton mentagrophytes*, *Aspergillus niger* and *Staphylococcus aureus*.

We claim:

1. Tin-organic compounds of the Formula I



wherein  $\text{R}_1$ ,  $\text{R}_2$ ,  $\text{R}_3$  and  $\text{R}_4$  are identical or different and represent alkyl radicals having 1 to 8 carbon atoms, phenyl radicals or phenyl radicals substituted by lower alkyl radicals and  $\text{R}_5$  represents hydrogen or the methyl group. 10

2. Tributyl tin- $\beta$ -tetrafluoro-cyclobutyl acrylate.
3. Tributyl tin- $\beta$ -methyl-tetrafluoro-cyclobutyl acrylate.
4. Triphenyl tin- $\beta$ -methyl-tetrafluoro-cyclobutyl acrylate.

References Cited

UNITED STATES PATENTS

|           |         |                 |           |
|-----------|---------|-----------------|-----------|
| 3,133,942 | 5/1964  | Hahl            | 260—429.7 |
| 3,409,652 | 11/1968 | Horrocks        | 260—429.7 |
| 3,651,107 | 3/1972  | Stanback et al. | 260—429.7 |

DANIEL E. WYMAN, Primary Examiner

A. P. DEMERS, Assistant Examiner

U.S. Cl. X.R.

160—15, 16; 117—47 A; 424—288